

## UNITED STATES PATENT OFFICE

1,935,875

STENCIL SHEET AND PROCESS FOR  
FORMING THE SAME

Louis E. Fuller, New York, N. Y.

No Drawing. Application March 19, 1932  
Serial No. 600,049

19 Claims. (Cl. 41—38.6)

My invention relates to permeable sheets so prepared as to be impervious to ink until pressure has been applied by means of raised characters such as the type of a writing machine, or by 5 means of a stylus, such part of the sheet thereby becoming pervious and so altered that ink will pass.

My invention may be used in place of and is an improvement over those stencil papers such as 10 wax and others which are easily ruptured in the typing process and which must be carefully handled to avoid injury to the coating. It is also an improvement over that class of stencil sheets requiring the application of moisture previous to 15 typing, in that while possessing to a marked degree the durability and toughness of such stencil sheets, and while capable of the same excellent and large number of reproductions, it does not require any moistening, this being a distinct ad- 20 vantage.

In general my new stencil sheet is distinguished over all other dry stencil sheets of which I have ever heard, by the fact that it may be bent, twisted and crushed repeatedly without impairment of its typing qualities and possesses great 25 chemical and mechanical stability. Suitably packed in cartons it will remain usable for long periods of time. In the typing process it also possesses the added improvement over other dry 30 stencil sheets in that it does not clog the type of the writing machine with extractive matter from the substance of the coating.

The object of my invention therefore is the production of an improved stencil sheet which shall 35 be tough and durable, which may be typed in a writing machine without moistening, will afford a large number of reproductions and will not deteriorate from long usage. A further object is that the stencil sheet shall be completely proof 40 against ink, this latter quality not being possessed by some of the stencil sheets that have been sold in the market. Unlike other stencil sheets except those requiring moistening prior to typing, my stencil sheet is proof against all neutral solvents 45 or solvents of ink, and in cases where they are kept for reprinting, may be cleansed from ink by means of benzine or oil or a similar substance, without any deterioration of the stencil sheet.

I accomplish this object by making use of the 50 great stability and other desirable properties of certain acid anhydrides when combined homogeneously in a film or coating with other stable substances such as hardened proteins or other colloids, and substances such as glycerin or its 55 equivalents, a concrete example of said formula

being given in the following description. When these substances are brought into solution by means of suitable solvents and applied to a sheet of open, fibrous material such as Japanese Yoshino paper, on evaporation of the solvents a 60 tough and impervious sheet results, which is capable of being typed in the ordinary manner. The acid anhydrides as made by my process and referred to, I have discovered are particularly adapted for use in stencil sheet coatings for the 65 reason that they are very stable and easily assimilated by the other ingredients of the film, the whole forming a tolerant mixture which deposits a homogeneous film of great flexibility and toughness. 70

The most useful of these acid anhydrides I have found, are those for the manufacture of which I have devised a special process, involving the use of a catalyst and relatively low temperatures, the final product being easy of purification. Anhydrides of the formula  $(R)_2O$  are obtained, the molecule of the acid or the acid containing substance being doubled if necessary. Acetic anhydride is used in molecular proportions, with an excess sufficient to remove the hydroxyl 80 from the acid, and to react on the  $C_3H_5$  radical in cases where glycerides are used. The material I prefer to employ is either stearic acid or a compound the principal constituent of which is stearic acid, such as commercial, hydrogenated 85 fatty oil. Such compound is a fatty oil containing more or less unsaturated fatty acids and which upon being hydrogenated or having hydrogen added to the acid radical, the fatty acids become saturated and thereby converted into 90 stearic acid. 75

In operating the process of forming my new stencil sheet therefore I first proceed to manufacture an acid anhydride by reacting on 280 parts of stearic acid and 3 parts of concentrated 95 sulphuric acid, and 90 parts of acetic anhydride, parts being by weight. The stearic acid is introduced warm, into a closed, acid proof container, and while in agitation the mixture of sulphuric acid and acetic anhydride is run in, heating 100 100 and agitation being continued for about one hour. The reaction takes place practically at atmospheric pressure and the temperature of the mix is maintained at from 120 to 140 degrees F. Double relief valves for the purpose of preventing material increase of pressure and formation of a partial vacuum are desirable for the container. 105

At the end of one hour a cold, saturated solution of brine is introduced, preferably heated to water- 110

bath temperature and agitation is continued for the purpose of washing the anhydride free of acids and impurities, this being repeated two or three times, each time the mixture being allowed to stand about fifteen minutes to allow the liquids to separate, the lower salt solution being then drawn off. At the third washing it is preferable to allow the mixture to stand about twelve hours as a more complete separation will be obtained.

10 After complete washing the warm, finished stearic anhydride is then drawn off, filtered and thus being freed from slight amounts of adhering salt by being allowed to stand in a warm condition, is ready for use.

15 The reaction product may also be freed from acids by other means such as neutralization of the sulphuric acid and distillation and recovery of the acetic acid formed, but the means of washing with brine I have found to be preferable.

20 I then prepare a mixture as follows, parts being by weight. Water 20 parts, denatured alcohol 60 parts, glacial acetic acid 10 parts, glycerine 40 parts, No. 1 ground gelatin 10 parts. This mixture is allowed to stand for about one hour to allow the gelatin to swell or may be agitated by suitable means to save time. The mixture is then warmed to about 100 degrees F. with agitation until the gelatin is dissolved. The solution 25 is then filtered, a suitable coloring matter being added if desired. There is then added to the above solution 40 parts of the anhydride of stearic acid warm, and dissolved in about 20 parts of benzine and 4 to 5 parts of formaldehyde, 30 this latter substance serving to harden the gelatin somewhat. The whole is then well agitated and again warmed if necessary to bring it to about 35 90 degrees F.

40 In the next step of my process the above solution is entered into a suitable pan or tray equipped with a scraping rod or straight-edge, the solution being maintained at around 80 to 90 degrees F. The sheets of Yoshino paper are then drawn over the surface of the solution, the surface being removed by the scraper, and suspended 45 to dry. On evaporation of the solvents the film sets to a homogeneous compound and in two or three hours the stencil sheets are ready for use.

50 Sheets are typed in the well-understood manner, being superimposed on heavy paper, a carrier sheet, and are then used in duplicating machines operated by inking pads or rollers for the purpose of making impressions.

55 The proportions of materials stated in the above solutions may be varied within reasonable limits for the adjustment of the character of the coating, it being understood that the proportion of gelatin, glycerin and acid anhydride are fixed substances that remain in the film to compose the coating of the stencil sheet. Less glycerin and anhydride for example will make a harder film and more a softer film. So that I do not bind myself to these stated proportions of solvents or other substances, it being understood 60 65 that my process broadly considered, consists of these substances or their equivalents for the purpose of a coating of predetermined character, solvents enough being used to give the necessary fluidity and limpidity to the solution. Part of the glacial acetic acid and also some of the alcohol may be replaced by water if desired. These matters will be readily understood by compounders or those skilled in the art.

70 In place of formaldehyde other hardening agents may be used such as various salts of

chromium or iron or other suitable metallic salts, as well as the alkaline chromates and dichromates. Or the hardening agent may be omitted if desired, the resulting sheet being somewhat softer in character.

80 In place of gelatin other protein bodies may be used if desired, in some cases more or less glycerin or acid anhydride being then desirable.

85 Glycerin being a polyhydric alcohol, equivalent substances such as other or similar alcohols may be used. In the compound film remaining in the coating of the stencil sheet it will be understood that the substances gelatin, hardened or otherwise, glycerin and acid anhydride, individually exercise an alternative or tempering effect on each other. The interaction of them produces the completed film possessing the necessary quality to be permeable in the typing operation.

90 In the manufacture of the acid anhydride other substances than hydrogenated fatty oil may be used, such as other glycerides or the acids themselves such as stearic, palmitic, oleic or mixtures of these, in each case the necessary molecular quantity of acetic anhydride plus the excess to react on the radical  $C_3H_5$  if any, being used. 95 These matters will be readily understood by those skilled in the art.

100 In the process above stated I may use an acid anhydride made by a different process such as heating in an autoclave for example, my invention 105 of the stencil sheet contemplating such acid anhydride as a necessary ingredient without regard to the process of manufacture.

110 By omitting the glycerin in the formula above, I may produce a stencil sheet of hardened protein 110 and acid anhydride alone, more friable, but useful for special typing purposes, without detracting from the substantial part of my invention.

115 In the process for the manufacture of the acid anhydride above described, I may use other catalysts than sulphuric acid, such as an acid, metallic salt, an oxide, or a catalyst similar to Twitchell's reagent. In fact I may use any suitable catalyst having the power to open the molecule of the acid reacted upon and maintain the 120 reaction. The glycerides referred to above means the ordinary fats and oils, containing fatty acids such as those stated, which may also be fatty oils which have had hydrogen added to the molecule, thus becoming more or less saturated compounds 125 such as stearin. The acids mentioned such as stearic, palmitic and oleic are higher fatty acids and my invention comprehends these or their equivalents.

130 It will be understood that the invention of the stencil sheet is not limited to the details as above described but that it comprehends broadly a stencil sheet adapted to be converted into a stencil by pressure, as by impact of type or a stylus thereon, it being essentially a fibrous base 135 provided with a coating which includes suitable anhydrides of the fats and fatty oils or their equivalents, this being so modified as to make it substantially stable for the purpose designed and responsive to pressure for the production of stencil 140 openings of character suitable for the passage of ink.

145 The invention of the process described herein is not limited to the precise details set forth but comprehends broadly the preparation of the acid anhydride described and compounding it with the remaining ingredients and impregnating open, fibrous material with the completed solution and drying, by suitable, equivalent means.

150 What I claim is:

1. A stencil blank convertible into a stencil by impact of type and the like thereon, comprising open, fibrous material impregnated with protein and a higher fatty acid anhydride. 50
- 5 2. A stencil blank convertible into a stencil by impact of type and the like thereon, comprising open, fibrous material impregnated with protein, a higher fatty acid anhydride and glycerin. 80
- 10 3. A stencil blank convertible into a stencil by impact of type and the like thereon, comprising open, fibrous material impregnated with protein and stearic anhydride. 85
- 15 4. A stencil blank convertible into a stencil by impact of type and the like thereon, comprising open, fibrous material impregnated with protein, stearic anhydride and glycerin. 90
- 20 5. A stencil blank convertible into a stencil by impact of type and the like thereon, comprising open, fibrous material impregnated with gelatin and a higher fatty acid anhydride. 95
- 25 6. A stencil blank convertible into a stencil by impact of type and the like thereon, comprising open, fibrous material impregnated with gelatin a higher fatty acid anhydride and glycerin. 100
- 30 7. A stencil blank convertible into a stencil by impact of type and the like thereon, comprising open, fibrous material impregnated with gelatin and stearic anhydride. 105
- 35 8. A stencil blank convertible into a stencil by impact of type and the like thereon, comprising open, fibrous material impregnated with gelatin, stearic anhydride and glycerin. 110
- 35 9. A stencil blank convertible into a stencil by impact of type and the like thereon, comprising open, fibrous material impregnated with hardened protein and a higher fatty acid anhydride. 115
- 40 10. A stencil blank convertible into a stencil by impact of type and the like thereon, comprising open, fibrous material impregnated with hardened protein and stearic anhydride. 120
- 45 11. A stencil blank convertible into a stencil by impact of type and the like thereon, comprising open, fibrous material impregnated with hardened protein, a higher fatty acid anhydride and glycerin. 125
- 50 12. A stencil blank convertible into a stencil by impact of type and the like thereon, comprising open, fibrous material impregnated with hardened protein, stearic anhydride and glycerin. 130
- 55 13. The process of forming a stencil sheet, consisting of heating and agitating a higher fatty acid or a higher fatty acid containing sub- 135
- stance with a dehydrating agent and a catalyst until dehydration of the acid occurs, removing the acids from the resulting acid anhydride, adding thereto protein dissolved in glycerin and suitable solvents and a hardening agent, impregnating an open, fibrous material with the said solution and drying. 140
14. The process of forming a stencil sheet, consisting of heating and agitating stearic acid with acetic anhydride and concentrated sulphuric acid, as a catalyst until dehydration of the stearic acid occurs, removing the acids from the resulting acid anhydride, adding thereto a solution of gelatin in suitable solvents and a hardening agent, impregnating an open, fibrous material with the solution and drying. 145
15. The process of forming a stencil sheet consisting of heating and agitating stearic acid with acetic anhydride and a catalyst such as concentrated sulphuric acid until dehydration of the stearic acid occurs, washing the resulting stearic acid anhydride with brine, adding benzine and a solution of gelatin and glycerin and a hardening agent, impregnating an open, fibrous material with the compound and drying. 150
16. The process of forming a stencil sheet involving the production and purification of a higher fatty acid anhydride, dissolving in benzine, adding to a solution containing protein and glycerin, impregnating a sheet of open, fibrous material with the solution and drying the sheet. 155
17. The process of forming a stencil sheet involving the production of a higher fatty acid anhydride, washing the same with brine, dissolving in benzine, adding gelatin, suitable solvents and a hardening agent, impregnating an open, fibrous material with the solution and drying. 160
18. The process of forming a stencil sheet involving the production of a higher fatty acid anhydride, dissolving the acid anhydride in a solution containing gelatin, glycerin, suitable solvents and a hardening agent, and impregnating an open, fibrous material with the solution and drying. 165
19. The process of forming a stencil sheet involving the production of a higher fatty acid anhydride and dissolving the same in a solution containing protein and glycerin and suitable solvents, coating the solution on fibrous material and drying. 170
- LOUIS E. FULLER.
- 60 135
- 65 140
- 70 145
- 75